

## UNITED STATES PATENT OFFICE

HANS SIMON, OF HANOVER, GERMANY, ASSIGNOR TO GÜNTHER WAGNER, OF HANOVER, GERMANY, A CORPORATION OF GERMANY

## STENCIL SHEET

No Drawing.

Application filed August 30, 1932. Serial No. 631,099.

This invention relates to improvements in stencil sheets.

Stencil sheets have been prepared by coating lace-like fibrous and porous sheets of paper, such as Japanese Yoshino paper, with plastic materials impervious to ink. These materials should be of sufficient softness and plasticity, or should be readily convertible into such condition as would permit the formation of open spaces in said sheet upon pressure, as by typewriter key, through which ink might pass.

Among the plastic materials advantageously utilized are proteins, such as glue or gelatin, which proteins are preferably suitably hardened, toughened, or coagulated to increase their durability and decrease their tackiness. With such plastic materials it is also desirable to use softening agents, such as glycerin, sugar, fats, oils and fatty acids and organic esters as well as filling materials of organic or inorganic nature, such as for example wood flour, bentonite and kieselguhr. These latter materials are desirably utilized to prevent sweating out of the softening materials and to decrease the adhesive properties of the sheet.

However, stencil sheets coated in this manner are not of as high tensile strength and durability as desirable, are influenced by adverse weather conditions and particularly tend to deteriorate rapidly if stored in hot and moist climates.

Furthermore glycerin, sugar and other polyhydroxy materials are not altogether completely satisfactory as plasticizers. When fat or fatty acid materials were utilized whether of animal, vegetable or mineral origin, the coating also is not very durable and tends to be readily influenced by weather conditions.

An object of this invention is to provide a stencil sheet provided with a plastic coating, preferably consisting of a protein material, which will be of high tensile strength and of great durability, which will not be influenced by adverse weather conditions and which may be stored safely for considerable periods in hot and moist climates.

A further object is to provide a stencil

sheet, the coating of which will have the desirable characteristics of a coating plasticized with fats, oils and/or fatty acids without any decrease in durability or liability to be greatly influenced by weather conditions. 55

In the preferred embodiment of the present invention the above and other objects of the present invention are realized by employing high molecular alcohols, whether saturated or unsaturated, and if desired, by including with these alcohols the aromatic phosphoric acid derivatives, as ingredients in the coating.

Among the alcohols which may be used are lauryl alcohol, myricil alcohol, and oleic 65 alcohol. These alcohols may be used singly, or in mixtures, preferably with the addition of phenolic esters of the phosphoric acid. Although the aliphatic alcohols specifically described are preferred, other high molecular 70 weight alcohols may be employed if of satisfactory properties containing substituent, such as halogen, nitro and aryl radicals, and so forth. In the case of high molecular weight aliphatic alcohols, these alcohols may 75 have straight or branch carbon chains, and may either be saturated or unsaturated. Generally the tricresyl ester of phosphoric acid (tricresyl phosphate) has been found to be most satisfactory as an additional plasticizing agent. 80

To give one specific example of a coating composition, the following composition has been utilized and found to be satisfactory:

|                     | Parts by weight |
|---------------------|-----------------|
| Gelatin             | 8               |
| Glycerin            | 3               |
| Tricresyl phosphate | 20              |
| Oleic alcohol       | 10              |
| Myricil alcohol     | 5               |
| Sulphonated oil     | 40              |
| Wood flour          | 6               |
| Pigment             | 10              |
| Dinitrotoluene      | 0.5             |
| Water               | 130             |

This coating composition may be conveniently applied by brushing or flowing it upon the paper sheet, or by dipping the sheet into 100

the coating solution, and if desired the coating composition may be in several operations. When being coated the sheet may be allowed to dry.

6 The sulphonated oil is preferably not of the type derived from marine sources. The pigment may desirably include ultramarine blue, while for wood flour the beechwood has been most conveniently utilized.

10 A hardening, toughening or coagulating agent may be suitably added to the coating, preferably by way of a second treatment, and preferably it is accomplished by treating the initial coating before drying with gaseous formaldehyde or with a small amount of a commercial formaldehyde solution. Other coagulating, toughening and hardening agents may also be employed.

20 Other plastic protein or nitrogenous material having similar characteristics to gelatin, and other similar coagulatable materials may also be employed alone or in combination with the gelatin. Instead of dinitrotoluene, other preserving agents may be employed.

What is claimed is:

1. A coating for stencil sheets, comprising a sulphonated oil, tricresyl phosphate, myricyl alcohol, gelatin, glycerin, wood dust, a pigment and a preservative.
2. A coating for stencil sheets, comprising tricresyl phosphate, oleic alcohol, gelatin and dinitrotoluene.
3. A coating for stencil sheets, comprising tricresyl phosphate, lauryl alcohol, gelatin and glycerin.
4. A coating mixture for making stencils, comprising 130 parts by weight of water, 40 parts by weight of a sulphonated oil, 20 parts by weight of tricresyl phosphate, 10 parts by weight of ultramarine blue, 10 parts by weight of oleic alcohol, 8 parts by weight of gelatin, 6 parts by weight of beechwood flour, 5 parts by weight myricyl alcohol, 3 parts by weight glycerin, and 0.5 parts by weight of dinitrotoluene.

In testimony whereof I have affixed my signature.

HANS SIMON.

20

95

25

100

30

105

35

110

40

115

45

120

50

125

55

130

60